

## UNITED STATES PATENT OFFICE

2,364,921

## LEADED MOTOR FUELS

Edward C. Shokal, Oakland, Calif., assignor to  
 Shell Development Company, San Francisco,  
 Calif., a corporation of Delaware

No Drawing. Application July 6, 1942,  
 Serial No. 449,964

8 Claims. (Cl. 44—69)

This invention relates to improved motor fuels containing a tetra-alkyl-lead. More particularly, my invention relates to tetra-ethyl-lead treated fuels containing as scavengers small amounts of certain tri-halogen alkanes having 2 to 5 carbon atoms.

When fuels containing only tetra-ethyl-lead are burned in an internal combustion engine, a deposit of lead compounds tends to accumulate in various parts of the combustion chamber, e. g., the spark plugs, valve stems, etc. This lead may cause severe deterioration of the effective parts, resulting in failure of spark plugs, sticking of valves, etc. Scavenger fluids for tetra-ethyl-lead, such as certain halogenated compounds, e. g., alkyl mono- or dichlorides or bromides, particularly ethylene dichloride, ethylene dibromide or mixtures of the compounds, are always incorporated into leaded fuels. The scavengers reduce lead deposits by releasing halogens during combustion which react with the lead to form volatile lead halides which are withdrawn from the combustion chamber with the products of combustion during the exhaust stroke.

The disadvantages of the aforesaid halogenated compounds are that they require a considerable excess of halogen to form, with substantially all of the lead, volatile compounds capable of being eliminated from the combustion chambers during operation of the engines. In the absence of sufficient halogen, lead deposits are formed on the porcelain and the electrodes of spark plugs, which deposits corrode the electrodes and eventually grow to such dimensions that the spark plugs are shorted and rendered useless. On the other hand, excess halogen causes marked corrosion and tends to "chew" away metal parts such as spark plug electrodes, valve seats, valve stems, cylinder walls, etc.

Another disadvantage of the currently used dihalogen compounds is that they boil at temperatures considerably lower than the boiling temperature of tetra-ethyl-lead, as shown by the examples in the table below:

|                                    | B. P., ° C. | At mm. Hg |
|------------------------------------|-------------|-----------|
| Ethylene dichloride.....           | 83          | 760       |
| Ethylene dibromide.....            | 131         | 760       |
| Tetra-ethyl-lead..... <sup>1</sup> | 200         | 760       |

<sup>1</sup> Decomposes.

As a consequence, these halogen compounds vaporize far more rapidly than tetra-ethyl-lead which leads to even greater excess of halogen in

some of the cylinders of multi-cylinder engines with a deficiency of halogen in other cylinders.

It is, therefore, an object of this invention to produce motor fuel mixtures in which the boiling temperature of the halogen compound is so nearly the same as that of the anti-knock agent that the constituents of the fuel are more uniformly vaporized and distributed. Another object is to prepare fuel mixtures, which, upon burning, leave a cleaner engine combustion chamber relatively free from lead deposits and corrosive substances. Another object is to produce fuel mixtures which contain halogen in amounts not more and preferably less than the stoichiometric equivalent of lead contained in the fuel and which, upon burning, still maintain a relatively clean engine. Still another object is to produce fuel mixtures having less tendency to corrode parts of internal combustion engines than leaded gasolines now available.

I have discovered that the above-enumerated objects can be accomplished by combining, in a motor fuel containing lead, a small amount of a chloro- or chloro-bromo hydrocarbon containing three halogen atoms and at least two and not more than five carbon atoms. Straight chain hydrocarbons are preferred. It is desirable to use these trihalogen hydrocarbons as the sole scavengers, i. e., not in admixture with those halogen hydrocarbons heretofore employed.

The stoichiometric equivalent as herein defined is the amount of halogen required to combine with lead according to the equation:

35       $2\text{Hal.} + \text{Pb} \rightarrow \text{Pb}(\text{Hal})_2$

The halogen atoms may be attached to any of the carbon atoms of the hydrocarbons, but preferably are attached to two adjacent primary and/or secondary carbon atoms as, for example, 40 in the preferred compounds 2-chloro-2,3-dibromo-butane and 2,2,3-tri-chloro-butane. 45 Tri-halogen aliphatic compounds, other than the above butanes, which are useful for my purposes are tri-chloro-ethanes, tri-chloro-propanes, such as 1,2,3-tri-chloro-propane, 1,2,2-tri-chloro-propane, 2,3,3-tri-chloro-propane, etc., tri-chloro-butanes such as 3,3,4-tri-chloro-butane, 2,3,4-tri-chloro-butane, etc., tri-chloro-pentanes, tri-chloro cyclopentane, corresponding methyl and ethyl substituted tri-chloro-propanes, butanes and pentanes; mixed-chloro-bromo compounds such as mono-chloro-dibromo-ethanes, propanes, butanes and pentanes, dichloro-mono-bromo-ethanes, propanes, butanes and pentanes of which the following are a few examples: 1,2-

dichloro - 2 - bromo - propane, 1 - chloro - 2,3-dibromo - propane, 1-chloro-1,2-dibromo-propane, 3-chloro-2,3-dibromo-propane, etc., 3-chloro-3,4-dibromo-butane, 2-chloro-3,4-dibromo-butane, 2,3-dichloro - 3 - bromo - butane, 1-chloro-2,3-dibromo-2-methyl propane, 1-chloro-2,3-dibromo-cyclopentane, 2-chloro - 2,3 - dibromopentane, 1-chloro-1,2-dibromo-3-methyl butane.

My compounds may be prepared by any known methods. One method is illustrated by the preparation of 2-chloro-2,3-dibromo-butane, as follows:

A sample of 2-chloro-butene-2, boiling between 60° C. and 70° C. was cooled to -35° C. The cool mixture was then strongly radiated with photo-flood lamps. Bromine under these conditions added to the unsaturated bond, rather than reacting by replacement of hydrogen. The ratio of components was 3 to 4 mols of 2-chloro-butene-2 to one mol of bromine. The bromine was vaporized and added in the vapor phase to the 2-chloro-butene-2 liquid with stirring. The resulting mixture was fractionated at reduced pressure. The product, 2-chloro-2,3-dibromo-butane was obtained as a liquid which boiled between 74° C. and 78° C. at 20 mm. pressure. The yield was 88%-90% of the theoretical calculated on the basis of bromine.

The amounts of my compounds which operate satisfactorily to supply the scavenging halogen necessary to keep the engine clean are generally those containing between .75 and 1.0 stoichiometric equivalents of halogen per the unit of lead present in the fuel. I prefer to use an amount of scavenger not in excess of the stoichiometric equivalent, although slightly greater amounts may be used if found necessary under severe engine conditions.

By using less than the stoichiometric equivalent of halogen, less or no free halogen will be present in the combustion chamber, and as a result corrosion of many inside parts of the engine is reduced materially. This reduction in corrosion is accomplished without sacrificing lead scavenging efficiency.

The invention is further illustrated by the following example:

*Example*

A sample of a commercial gasoline was divided into five portions. This fuel contained 4 cc. of tetra-ethyl-lead per gallon. To portion 2 was added 2-chloro-2,3-dibromo-butane in an amount capable of supplying halogen equal to 1/2 of the stoichiometric equivalent of the lead present. To portion 3 was added 2-chloro-2,3-dibromo-butane in an amount capable of supplying halogen equal to 3/4 of the stoichiometric equivalent of the lead present. To portion 4 was added 2-chloro-2,3-dibromo butane in an amount capable of supplying halogen equal to the stoichiometric equivalent of the lead present. To portion 5 was added an amount of "Motor Mix" (25.4 wt.% ethylene dibromide and 74.6 wt.% ethylene dichloride) capable of supplying halogen equal to 1.15 of the stoichiometric equivalent of the lead present. (This amount of "Motor Mix" is standard in today's commercial automotive fuels containing lead.) Each of the resulting blends was run in a C. F. R. engine for 14 hours. At the end of

each run, the combustion chamber was inspected and then the deposit was collected and analyzed. Results were as follows:

|    | Composition of fuel<br>4 cc. T. E. L. per gal. | Condition of spark plug                                 |
|----|------------------------------------------------|---------------------------------------------------------|
| 5  | No added halogen.....                          | Heavy yellow deposit, center point corroded very badly. |
| 10 | 0.5 theory chloro-dibromo-butane.              | Porcelain yellow, center point corroded.                |
|    | 0.75 theory chloro-dibromo-butane.             | Porcelain clean, center point in good shape.            |
|    | 1.0 theory chloro-dibromo-butane.              | Entire spark plug looks like a new one.                 |
|    | Commercial Motor Mix (1.15 theory halogen).    | Yellow stain on porcelain, center point in good shape.  |

15 The above data show that the spark plug porcelain condition is better with from roughly 15% to 40% less halogen, when using applicant's compounds, than when using the compounds currently in use.

20 I claim as my invention:

1. A leaded gasoline containing a compound selected from the group of chloro and chloro-bromo alkanes containing 3 halogen atoms per molecule and at least 2 and not more than 5 carbon atoms the amount of the added halide being sufficient to reduce the deposit of lead compounds formed on combustion of the gasoline.
2. The gasoline of claim 1 wherein the alkane 30 is a straight chain hydrocarbon.
3. A leaded gasoline containing a mono-chloro-di-bromo hydrocarbon containing at least 2 and not more than 5 carbon atoms the amount of the added halide being sufficient to reduce the deposit of lead compounds 35 formed on combustion of the gasoline.
4. A leaded gasoline containing a tri-halogen compound selected from the group of chloro and chloro-bromo alkanes containing at least 2 and not more than 5 carbon atoms, two of which halogen atoms are attached to the same carbon atom the amount of the added halide being sufficient to reduce the deposit of lead compounds formed on combustion of the gasoline.

45 5. A leaded gasoline containing a tri-halogen compound selected from the group of chloro and chloro-bromo alkanes containing at least 2 and not more than 5 carbon atoms, said halogens being attached to two adjacent carbon atoms the amount of the added halide being sufficient to reduce the deposit of lead compounds formed on combustion of the gasoline.

6. A leaded gasoline containing 2-chloro-2,3-dibromo-butane the amount of the added halide being sufficient to reduce the deposit of lead compounds formed on combustion of the gasoline.

7. A leaded gasoline containing 2,2,3-trichloro-butane the amount of the added halide being sufficient to reduce the deposit of lead compounds formed on combustion of the gasoline.

8. A leaded gasoline containing an amount of a compound selected from the group of chloro and chloro-bromo alkanes containing 3 halogen atoms per molecule and at least 2 and not more than 5 carbon atoms, said amount containing halogen in quantities equal to between .75 and 1.0 stoichiometric equivalents of the lead contained in said gasoline.

EDWARD C. SHOKAL.